

F. EBERHART.

METHOD OF MANUFACTURING INTERIORLY COATED CANS.

APPLICATION FILED SEPT. 9, 1912.

1,094,840.

Patented Apr. 28, 1914.

Fig. 1 17 16 15



Fig. 2



Fig. 3 25



Witnesses:

Wm. Geiger  
Pearl Abrams.

Inventor:

Felix Eberhart  
By Munday Evans, Adcock & Clarke  
his Atty's

# UNITED STATES PATENT OFFICE.

FELIX EBERHART, OF NEWARK, NEW JERSEY, ASSIGNOR TO AMERICAN CAN COMPANY, OF NEW YORK, N. Y., A CORPORATION OF NEW JERSEY.

## METHOD OF MANUFACTURING INTERIORLY-COATED CANS.

1,094,840.

Specification of Letters Patent. Patented Apr. 28, 1914.

Application filed September 9, 1912. Serial No. 719,369.

To all whom it may concern:

Be it known that I, FELIX EBERHART, a citizen of the United States, residing in Newark, in the county of Essex and State 5 of New Jersey, have invented a new and useful Improvement in Methods of Manufacturing Interiorly-Coated Cans, of which the following is a specification.

This invention relates to improvements in 10 method of manufacturing interiorly coated cans.

An object of the invention is to provide a process wherein the lacquer or other coating material which is employed to coat the interior 15 of cans is utilized as the sealing or packing compound in the seam formed between the can end and body, the end and body being seamed or joined together while the lacquer or other protective coating material 20 is in a soft, more or less fluid or plastic condition.

The invention furthermore consists in the improvements in the steps and the novel combinations of the steps of the process 25 as more particularly described or claimed hereinafter.

In the drawing forming a part of this specification are illustrated various mechanisms adapted to carry out my improved 30 process, and in said drawing, Figure 1 denotes a part sectional view of a portion of a machine adapted to spray or coat can ends with lacquer or other protective coating material. Fig. 2 represents a portion of a 35 double seaming machine, parts being broken away to more clearly illustrate the construction, and Fig. 3 is a sectional view of a baking or drying apparatus employed for drying or hardening the lacquer or other 40 coating material after the can body and end have been united.

In the drawing, 10 denotes the table or platform of a spraying or coating machine suitable for applying lacquer or other coating 45 material to can ends, and over said table or platform, as shown in the drawing, is adapted to run an endless conveyer 11 provided with can end holding chucks 12 in which are adapted to be seated can ends 13, 50 the latter being sprayed with the lacquer or other coating material as they pass beneath the spraying nozzle 14, which is supplied with the lacquer or other equivalent material through a pipe 15 leading to a supply 55 tank (not shown), the lacquer or other ma-

terial being forced through the perforations 16 in the nozzle by means of compressed air supplied through a pipe 17 connected to a suitable source of compressed air (not shown). During this step of the process, 60 the coating material is applied to the entire upper surface of the can end, including the can end flange which forms part of the double seam. While the coating material is soft or in a more or less liquid or plastic 65 condition, the can end is loosely united to a can body 18, the latter being formed preferably from a previously lacquered or coated sheet and flanged in the usual manner. The loosely assembled can body and end are then 70 placed in the seaming machine 19 between the chucks 20 and 21, and double-seamed by the seaming rollers, one of which is shown at 22 and adapted to be operated by a cam 23 in a well known manner. After 75 the can body and end have been united by the seamer, the can is then placed on an endless conveyer 24 and passed through a drying or baking oven 25 to thereby dry or 80 harden the lacquer or other equivalent protective coating material.

The mechanisms shown in the drawing and described, represent merely well known forms for carrying out the process, but it will be evident that the lacquer or coating 85 material might be applied in other ways, and also that the ends and bodies might be united by seams of other form than double seams. Furthermore, the process is not limited to the employment of lacquer or coating material which must be dried or baked, 90 since the process could be carried out by using substances which dry and harden spontaneously, or which may even be "flashed", the process remaining the same 95 so long as the coating material is adapted to serve both as a protective coating and as a sealing or packing compound.

The advantages resulting from the employment of my improved process are many, 100 and among them may be noted the following: By uniting the can end, with the coating material in a soft or unhardened condition, to the can body, all danger of scratching or marring the lacquer on the 105 can end is thus avoided. Hitherto where the can heads have been lacquered or otherwise provided with a protective coating, and shipped in quantities and fed from stacks, the lacquer or coating has been liable 110.

to injury from scratching and marring. With my improved process, the lacquer or other compound used for coating is evenly distributed throughout one entire surface of the can end, including the seam-forming flange, which results in an even distribution of the material throughout the entire seam, whereas hitherto in the old process, where the "dope", sealing or packing material has been applied to the can end seaming flanges and dried, it has been found that the sealing or packing material, during the drying step, runs and collects unevenly in the groove, with the result that portions of the seam are unprovided with any sealing compound at all.

I claim:

1. The method of manufacturing interiorly coated, seamed cans which consists in coating the entire surface of a can end, including its seam forming flange, with a combined protective and seal-forming coating material, then assembling the coated can end, while the coating material is still soft, with a flanged can body having a hardened protective coating on its interior, and then seaming said can end and can body before the coating material in the joint has hardened.

2. The method of manufacturing interiorly coated, seamed cans which consists in the coating one entire surface of a can end, including its seam forming flange, with a combined protective and seal-forming coating material, then assembling the coated can end, while the coating material is still soft, with a flange can body having a hardened protective coating on its interior, then seaming said can end and can body before the coating material in the joint has hardened, and finally subjecting the seamed can to a drying or baking operation.

3. The method of manufacturing interiorly coated, seamed cans which consists in coating a can end with a combined protective and seal-forming coating material, then assembling the coated can end, while the coating material is still soft, with a flanged can body made from previously coated plate and then seaming the can end and body together.

4. The method of manufacturing interiorly coated, seamed cans which consists in coating a can end with a combined protec-

tive and seal-forming coating material, then 55 assembling the coated can end, while the coating material is still soft, with a flanged can body made from previously coated plate, seaming the can end and body together and finally subjecting the seamed can to a dry- 60 ing or baking operation.

5. The method of manufacturing interiorly coated, seamed cans which consists in coating a can end with a combined protective and seal-forming coating material, 65 then assembling the coated can end, while the coating material is still soft, with a flanged can body having a hardened protective coating on its interior, and then seaming the can end and body together. 70

6. The method of manufacturing interiorly coated, double seamed cans which consists in coating a can end with a combined protective and seal-forming coating material, then assembling the coated can 75 end, while the coating material is still soft, with a flanged can body made from previously coated plate, and then double seaming the can end and body together.

7. The method of manufacturing interiorly coated, double seamed cans which consists in coating one entire surface of a can end, including its seam forming flange, with a combined protective and seal-forming coating material, then assembling the 80 coated can end, while the coating material is still soft, with a flanged can body having a hardened protective coating on its interior, and then double seaming the can end and can body before the coating material in the joint has hardened.

8. The method of manufacturing interiorly coated, double seamed cans which consists in coating one entire surface of a can end, including its seam forming flange, 85 with a combined protective or seal-forming coating material, then assembling the coated can end, while the coating material is still soft, with a flanged can body having a hardened protective coating on its interior, 100 then double seaming the can end and can body before the coating material in the joint has hardened, and finally subjecting the seamed can to a drying or baking operation.

FELIX EBERHART.

Witnesses:

W. D. FOSTER,  
C. W. GRAHAM.

Corrections in Letters Patent No. 1,094,840.

It is hereby certified that in Letters Patent No. 1,094,840, granted April 28, 1914, upon the application of Felix Eberhart, of Newark, New Jersey, for an improvement in "Methods of Manufacturing Interiorly-Coated Cans," errors appear in the printed specification requiring correction as follows: Page 2, line 32, before the word "coating" strike out the article "the"; same page, line 96, for the word "or" read *and*; and that the said Letters Patent should be read with these corrections therein that the same may conform to the record of the case in the Patent Office.

Signed and sealed this 26th day of May, A. D., 1914.

[SEAL.]

R. F. WHITEHEAD,  
*Acting Commissioner of Patents.*